

## UNITED STATES PATENT OFFICE

2,154,096

## LUBRICATING OIL

Clarence M. Loane, Hammond, Ind., assignor to  
Standard Oil Company, Chicago, Ill., a corpora-  
tion of Indiana

No Drawing. Application November 16, 1936,  
Serial No. 111,684

## 7 Claims. (Cl. 87-9)

This invention relates to lubricants and, in particular, to addition agents imparting improved properties to lubricants.

This invention has particular utility in improving the lubricating properties of lubricating oils and/or in preventing or inhibiting the corrosion of "hard metal" alloy bearings such as copper-lead, cadmium-nickel and cadmium-silver bearings which, to a large extent, have replaced soft metal bearings, such as Babbitt metal, in the trend toward internal combustion engines having high compression ratios and increased acceleration and increased speed characteristics. The use of the "hard metal" bearings has created lubricating and corrosion problems, particularly in connection with highly refined oils, some of which may be very corrosive to bearings of the hard metal type.

As used herein "highly refined" lubricating oil means viscous oils which have a minimum viscosity of S. A. E. 10 oils, or higher, and which have been subjected to such refining processes that the paraffinicity of the oil is markedly increased. It has been found that "highly refined" lubricating oils cause corrosion to alloy bearings of the hard metal type such as cadmium-silver alloy bearings to the extent of about 5 mg/cm.<sup>2</sup> and even greater when such bearings are submerged for 25 hours or less in an air agitated oil which has been preoxidized at about 340° F. for 25 to 50 hours. The motor oils may be "highly refined" lubricating oils as such or mixtures of highly refined lubricating oils with less highly refined lubricating oils, or stated in another way, mixtures of corrosive oils and non-corrosive oils, examples of the latter being lubricating oil fractions from Winkler Crude or crudes of the Winkler type.

I have found that corrosion of alloy bearings of the cadmium-silver type can be inhibited and highly desired properties can be imparted to lubricating oils by adding thereto up to 2%, but preferably 0.05% to 0.75%, of certain organic materials, particularly monovalent radical substituted heterocyclic organic compounds selected from the group consisting of thiazines having the general formula

50



55

and thiazoles having the general formula



in which R may be substituted alkyl and/or aryl and/or aralkyl and/or amino and/or amino alkyl and/or alkyl substituted amino and/or mercapto and/or alkyl mercapto and/or aryl mercapto radical or radicals.

The term thiazole as used herein includes the thio monazoles, the (1-2-3, 1-2-4, 1-2-5, and 1-3-4) thio diazoles and the (1-2-3-4 and 1-2-3-5) thio triazoles. I may also use the corresponding hydro thiazines and thiazoles.

Examples of the compound I may use are:

2-amyl thiazole  
 4-amyl thiazole  
 5-amyl thiazole  
 2,4 dihexyl thiazole  
 2,5 dihexyl thiazole  
 4,5 dihexyl thiazole  
 Trimethyl thiazole  
 Tributyl thiazole  
 5-phenyl thiazole  
 Triphenyl thiazole  
 4-propyl 2-amino thiazole  
 4-phenyl 2-amino thiazole  
 2-phenyl amino thiazole  
 4-butyl 2-phenylamino thiazole  
 4-hexyl 2-mercapto thiazole  
 5-phenyl 2-mercapto thiazole  
 2-butyl 4,5 dihydro thiazole  
 4-amyl 2-mercapto thiazoline  
 2-methyl thiazoline  
 2-phenyl thiazoline  
 Meta thiazine  
 Mu-phenyl penthiazoline  
 Mu-phenyl-alpha-dimethyl-gamma-methyl  
 penthiazoline  
 Mu-mercapto-gamma-methyl penthiazoline  
 Mu-mercapto-gamma-butyl penthiazoline  
 Gamma-methyl-alpha-dimethyl penthiazole  
 line  
 Para thiazine  
 2,4 dibutyl thiazine

Some of the foregoing compounds may not be completely soluble in the lubricant, in which case effective results are obtained by suspending the inhibitor in the lubricant by means of small amounts of a peptizing agent such as aluminum naphthenate, aluminum stearate, etc.

When highly refined motor oils are used in internal combustion engines provided with bearings of the cadmium-silver and copper-lead type the bearings, after a comparatively short time, fall due to the corrosion of the bearing metal. This is probably due to the removal of certain constituents from the oil which behave as corrosion inhibitors. I have found that when small amounts, for example up to 2%, but preferably 0.05% to 0.75%, of the foregoing compounds are added to highly refined lubricating oils the life of the "hard metal" alloy type bearings is markedly increased and in most cases difficulties due to corrosion are entirely avoided.

15 I claim:

1. The method of preventing corrosion of bearing metal alloys having the corrosive susceptibility of alloys of the group consisting of cadmium-silver alloys, cadmium-nickel alloys, and 20 copper-lead alloys, in the presence of highly refined lubricating oils normally corrosive to said bearings in internal combustion engines which comprises adding to said lubricating oils in a small but sufficient proportion to substantially 25 retard said corrosion a monovalent radical substituted heterocyclic organic compound selected from the group consisting of thiazines having the general formula



in which R is a radical selected from the group consisting of alkyl, aryl, aralkyl, amino, amino alkyl, mercapto, alkyl mercapto and aryl mercapto radicals.

2. The method of preventing corrosion of bearing metal alloys having the corrosive susceptibility of alloys of the group consisting of cadmium-silver alloys, cadmium-nickel alloys and copper-lead alloys in the presence of highly refined lubricating oils normally corrosive to said bearings which comprises adding to said lubricating oils about 0.05% to about 0.75% of a monovalent radical substituted heterocyclic organic compound selected from the group consisting of thiazines having the general formula



and thiazoles having the general formula



in which R is a radical selected from the group consisting of alkyl, aryl, aralkyl, amino, amino alkyl, mercapto, alkyl mercapto and aryl mercapto radicals.

3. The method of preventing corrosion of bearing metal alloys having the corrosive susceptibility of alloys of the group consisting of cadmium-silver alloys, cadmium-nickel alloys and copper-lead alloys in the presence of highly refined lubricating oils normally corrosive to said bearings which comprises adding to said lubricating oils an alkyl thiazole in a small but sufficient proportion to substantially retard said corrosion.

4. The method of preventing corrosion of bearing metal alloys having the corrosive susceptibility of alloys of the group consisting of cadmium-silver alloys, cadmium-nickel alloys and copper-lead alloys in the presence of highly refined lubricating oils normally corrosive to said bearings which comprises adding to said lubricating oil from about 0.05% to about 0.75% of a tributyl thiazole.

5. The method of preventing corrosion of bearing metal alloys having the corrosive susceptibility of alloys of the group consisting of cadmium-silver alloys, cadmium-nickel alloys and copper-lead alloys in the presence of highly refined lubricating oils normally corrosive to said bearings which comprises adding to said lubricating oils an aryl thiazole in a small but sufficient proportion to substantially retard said corrosion.

6. The method of preventing corrosion of bearing metal alloys having the corrosive susceptibility of alloys of the group consisting of cadmium-silver alloys, cadmium-nickel alloys and copper-lead alloys in the presence of highly refined lubricating oils normally corrosive to said bearings which comprises adding to said lubricating oil from about 0.05% to about 0.75% of a triphenyl thiazole.

7. The method of preventing corrosion of bearing metal alloys having the corrosive susceptibility of alloys of the group consisting of cadmium-silver alloys, cadmium-nickel alloys and copper-lead alloys in the presence of highly refined lubricating oils normally corrosive to said bearings which comprises adding to said lubricating oil from about 0.05% to about 0.75% of a mercapto thiazole.

CLARENCE M. LOANE. 60